

## UNITED STATES PATENT OFFICE

2,617,771

## CORROSION RETARDER

John T. Rucker, Lewiston, N. Y., assignor to  
Hooker Electrochemical Company, Niagara  
Falls, N. Y., a corporation of New York

No Drawing. Original application September 27,  
1946, Serial No. 699,640, now Patent No.  
2,459,119, dated January 11, 1949. Divided and  
this application July 30, 1948, Serial No. 41,727

4 Claims. (Cl. 252—149)

## 1

My invention relates more particularly to retarders of corrosion of metals by acids.

It is known that certain substances exert a protective effect upon metals, against attack of acids thereon, by rendering the metal passive with respect to the acid, i. e., as anti-catalysts. I will refer to these hereinafter as "inhibitors." It is also known that certain other substances exert a protective effect by interposing a film between the metal and the acid. These are of the nature of detergents, or dispersing or wetting agents, characterized by low surface tension. I will refer to these hereinafter as "surface active" materials.

Among the agents of the inhibitor category are the aralkyl thio-cyanates, such as benzyl and cymene thio-cyanates. These are typical examples of aralkyl thio-cyanates, each having a methyl group, to which the thio-cyanate group is attached, and the cymene having, in addition, a propyl group. However, these compounds are of low solubility in acid pickling baths. Also, benzyl thio-cyanate has not only an exceedingly disagreeable odor, but toxic and lachrymatory properties, the effects of which are aggravated by its low solubility and consequent tendency to collect at the surface of the bath and spatter into the atmosphere. For these reasons, these compounds have heretofore had little importance, except under conditions permitting of vigorous agitation.

Among the agents of the surface active category are the quaternary ammonium compounds, such as lauryl pyridinium chloride and lauryl dimethyl benzyl ammonium chloride. These are selected examples of quaternary ammonium compounds in which the nitrogen is in the ring and chain respectively. They are not only quite soluble in acid pickling baths, but also have the property of increasing the solubility of other organic compounds, including the thio-cyanates. When used in pickling baths, their saponaceous character causes them to form a foam layer upon the surface.

The effectiveness of these surface active materials is illustrated by the following examples, in which the abbreviations "LPC" and "LDBAC" stand for lauryl pyridinium chloride and lauryl dimethyl benzyl ammonium chloride respectively, and the expression "protection per cent" signifies

## 2

the extent to which the agent is effective in eliminating corrosion altogether:

## Example I

|   | Metal, steel | Acid, sulphuric, 15% | Temperature, 75° C. | Corrosion retarder         | None | LPC  | LDBAC |
|---|--------------|----------------------|---------------------|----------------------------|------|------|-------|
| 5 |              |                      |                     | Percent retarder by weight | —    | .02  | .02   |
|   |              |                      |                     | Weight loss per sq. c. m.  | —    | .048 | .0076 |
|   |              |                      |                     | per hour g.                | .119 | 60.0 | 93.6  |

10 It will be seen from the above examples that the addition of minute quantities of these materials to acid pickling baths greatly diminishes the attack upon steel.

I have now found that the analogous quaternary ammonium thio-cyanates, i. e., lauryl pyridinium thio-cyanate and lauryl dimethyl benzyl ammonium thio-cyanate, are very soluble in acid pickling baths, for practical purposes odorless and non-toxic and very effective as corrosion retarders.

15 This is illustrated by the following example, to which I have also added benzyl pyridinium thio-cyanate for comparison, and in which these compounds are denoted by the abbreviations 20 "LDBATC," "LPTC" and "BPTC" respectively:

## Example II

|    | Metal, steel | Acid, sulphuric, 15% | Temperature, 75° C. | Corrosion retarder                   | None | LDBATC | LPTC  | BPTC |
|----|--------------|----------------------|---------------------|--------------------------------------|------|--------|-------|------|
| 30 |              |                      |                     | Percent retarder by weight           | —    | .02    | .02   | .02  |
|    |              |                      |                     | Weight loss per sq. c. m. per hr. g. | .119 | .0047  | .0021 | .024 |
|    |              |                      |                     | Protection, percent                  | —    | 96.0   | 98.2  | 79.8 |

It will be seen by comparison Examples I and II 35 that these alkyl quaternary ammonium thio-cyanates are much more effective as retarders of corrosion than the corresponding chlorides. It will also be seen that these alkyl quaternary ammonium thio-cyanates are much superior to the

40 analogous aryl thio-cyanates. The superiority of the alkyl pyridinium thio-cyanates to benzyl pyridinium thio-cyanate is a surprising and unpredictable discovery, since, as shown above, benzyl thio-cyanate is one of the most effective 45 corrosion inhibitors known. Another surprising discovery is that, whereas lauryl dimethyl benzyl ammonium chloride is superior to lauryl pyridinium chloride, lauryl pyridinium thio-cyanate is decidedly superior to lauryl dimethyl benzyl ammonium thio-cyanate.

At room temperature, lauryl pyridinium thiocyanate is a greasy, semi-solid, of about the consistency of butter. It becomes wholly liquid at 90° C. Lauryl dimethyl benzyl ammonium thiocyanate is an oily liquid at room temperature.

In order to show that my corrosion retarders have exceptional properties, I present herewith a table showing the percentage of protection afforded by my compounds, as compared with a considerable number of the best known corrosion retarders, taken from "Chemical Industries," 1939, vol. 37, page 124, against 4 per cent sulphuric acid at 71° C.

|                                             | Wt. Percent | Protection, Percent |
|---------------------------------------------|-------------|---------------------|
| Triethylamine                               | 0.15        | 10.5                |
| Aniline                                     | 0.09        | 14.5                |
| Pyridine                                    | 0.08        | 19.0                |
| Quinoline                                   | 0.13        | 49.4                |
| Acridine                                    | 0.18        | 82.4                |
| 2-me-quinoline                              | 0.15        | 53.0                |
| me-acridine                                 | 0.20        | 81.8                |
| Phenyl acridine                             | 0.29        | 90.2                |
| Nitrogen bases                              | 0.1         | 88.                 |
| Lauryl pyridinium chloride                  | 0.1         | 85.                 |
| Lauryl dimethyl benzyl ammonium thiocyanate | 0.02        | 96.                 |
| Lauryl pyridinium thiocyanate               | 0.02        | 98.2                |
| Lauryl pyridinium thiocyanate               | 0.01        | 99.4                |

It will be seen from the above that lauryl dimethyl benzyl ammonium thiocyanate and lauryl pyridinium thiocyanate rank high among corrosion retarders, and when it is remembered that they have the advantage over most of them of high water solubility, non-toxicity, and freedom from offensive odor, their importance as corrosion retarders will be manifest.

Corrosion retarders are useful wherever acids are handled in metal equipment, of which pickling of metal is only one of many illustrations, acid treatment of oil wells being another. Another use of such retarders is in lubricants, which are liable to develop acidity through oxidation, by contact with air. Organic acids developed in lubricating oils, such as those used in automotive crankcases, are mild compared with pickling acids, but the time factor is measured in months, instead of hours, and in the long run the corrosive effect of such acids may be very serious, especially upon bearing alloys, such as those composed of lead, tin, copper and less common metals. It is difficult to give a quantitative measure of the effect of corrosion retarders in lubricating oils, as the matter is complicated by wear. Nevertheless,

visual comparison of the effects of lubricating oils upon bearings, with and without my retarders, indicates that my retarders have a useful effect in such oils.

While I have given examples of the results obtained with my compositions only in proportions ranging from 0.02 to 0.1 per cent by weight, I do not wish to be held to these limits, as my retarders are useful in proportions as low as .005 per cent, and there is no objection to using up to 5 per cent of the retarder.

This application is a division of my co-pending application, Serial Number 699,640 filed September 27, 1946, now Patent No. 2,459,119 issued January 11, 1949.

I claim as my invention:

1. A composition substantially non-corrosive to metals comprising a dilute aqueous solution of an inorganic acid and 0.005 to 5 per cent by weight of a quaternary ammonium compound selected from the group consisting of lauryl pyridinium thiocyanate and lauryl dimethyl benzyl ammonium thiocyanate.

2. A composition substantially non-corrosive to metals comprising a dilute aqueous solution of sulfuric acid and 0.005 to 5 per cent by weight of lauryl pyridinium thiocyanate.

3. A composition substantially non-corrosive to metals comprising a dilute aqueous solution of sulfuric acid and 0.005 to 5 per cent by weight of lauryl dimethyl benzyl ammonium thiocyanate.

4. The method of protecting metals against corrosion by dilute aqueous acids which comprises incorporating in the acid 0.005 to 5.0 per cent by weight of a quaternary ammonium compound selected from the group consisting of lauryl pyridinium thiocyanate and lauryl dimethyl benzyl ammonium thiocyanate.

JOHN T. RUCKER.

#### REFERENCES CITED

The following references are of record in the file of this patent:

#### UNITED STATES PATENTS

| Number    | Name                 | Date          |
|-----------|----------------------|---------------|
| 2,006,216 | MacArthur et al. --- | June 25, 1935 |
| 2,203,649 | Felkers -----        | June 4, 1940  |
| 2,254,940 | Endres -----         | Sept. 2, 1941 |
| 2,321,517 | Rosen -----          | June 8, 1943  |
| 2,340,996 | Smyers -----         | Feb. 8, 1944  |
| 2,402,526 | Pikl -----           | June 18, 1946 |